

May 14, 1957

R. J. MAS ET AL

2,792,077

## RECOVERY OF TITANIUM TETRACHLORIDE

Filed Jan. 18, 1956

2 Sheets-Sheet 1



INVENTEURS  
Robert J. Massé André L. Michaud

BY

*Follard, Johnston, Smythe & Robertson  
Atty's.*

May 14, 1957

R. J. MAS ET AL.

2,792,077

RECOVERY OF TITANIUM TETRACHLORIDE

Filed Jan. 18, 1956

2 Sheets-Sheet 2



FIG. 3



FIG.4

**INVENTORS**

Send André L Michaud

*Pollard, Johnston, Smythe & Robertson  
Atty's.*

1

2,792,077

## RECOVERY OF TITANIUM TETRACHLORIDE

Robert J. Mas, Thann, and Andre L. Michaud, Vieux-Thann, France, assignors to Fabriques de Produits Chimiques de Thann et de Mulhouse, Thann, France, a corporation of France

Application January 18, 1956, Serial No. 559,993

14 Claims. (Cl. 183—120)

The present invention relates to an improved process for separating normally solid components from titanium tetrachloride contained in hot chlorination gases produced by the chlorination of oxidic titaniferous materials.

As is known, titanium tetrachloride is obtained by the action of chlorine on oxidic titaniferous materials at high temperatures in the presence of reducing agents. Rutile, ilmenite, synthetically obtained concentrates, such as titaniferous oxidic slags, etc. may be used as raw materials. The hot or crude gases coming from the chlorinator, in addition to gaseous vapors of  $TiCl_4$ , contain normally gaseous materials, such as  $CO$ ,  $CO_2$ ,  $Cl_2$ , possibly nitrogen and volatilized normally solid metal chlorides, such as ferric, possibly ferrous chlorides, and aluminum chloride. The vaporized metal chlorides may also include  $SiCl_4$  and chlorides of vanadium, zirconium, etc.

The separation of the technical grade titanium tetrachloride from the mixture essentially free of undissolved solids is a difficult task due to the formation of deposits on the walls of condensers, on pipes, on heat exchangers and other parts of the apparatus with a consequent clogging or blockage of the apparatus. These deposits are made up principally of normally solid metal chlorides which are only slightly soluble or insoluble in titanium tetrachloride such as, more particularly, ferric chloride and aluminum chloride. The deposits may contain also the dust contained in the gases formed in the chlorinator which flow therefrom at a fairly rapid rate.

Due to the difficulties involved, a number of processes for recovering the titanium tetrachloride obtained by the chlorination of oxidic titaniferous materials have been suggested. For the most part the suggested processes are of two types, namely:

(a) The chlorination gases are sprayed or scrubbed with cold titanium tetrachloride in such quantity that the larger part or substantially all of the titanium tetrachloride contained in the gases is condensed together with the normally solid chloride with a subsequent separation of the titanium tetrachloride, for instance, by distillation.

(b) The chlorination gases are sprinkled or bathed with titanium tetrachloride in such a small quantity that all or substantially all of the titanium tetrachloride present is removed in gaseous form. Thus the condensed solid chlorides are separated either in the dry state or as a slurry containing a small proportion of liquid titanium tetrachloride.

Each of the two types of processes described is accompanied by serious disadvantages. In type "a," the titanium tetrachloride recovered comes from the condensed titanium tetrachloride which is contaminated by the solid chlorides from which it must be separated through a rather costly process. The condensation is obtained through the utilization of the sensible heat of cold or cool titanium tetrachloride which requires a large flow of liquids and consequently large size heat exchangers are required. It is necessary, also, to use large size coolers and such apparatus working on turbid liquors, are always

2

subject to clogging and thus do not function very satisfactorily.

In type "b," the usual type of heat exchangers cannot be used since the danger of stoppage due to the deposit of dry solid chlorides is too great. Therefore, it is necessary to atomize the titanium tetrachloride in order to obtain a good heat exchange. Furthermore, it is necessary to have an almost pure titanium tetrachloride for atomization, for otherwise the atomizers may become clogged. Apart from the foregoing difficulties encountered in atomizing the titanium tetrachloride, the technique for using atomizers is inherently an exact one and does not assure a thorough washing of the chlorination gases. Consequently part of the solid chlorides remain in the chlorination gases or vapors and the subsequently recovered titanium tetrachloride is not very pure. It is difficult also to remove dry chlorides or the slurry of chlorides which deposit at the base of the tower containing the atomizer. Normally one needs special equipment, such as scrapers or chains, requiring costly maintenance.

This invention has as a principal object a process for the recovery of technical grade titanium tetrachloride from the chlorination gases obtained from oxidic titaniferous materials which is simple in operation and requires simple and inexpensive apparatus and thereby leads to lower processing costs. The invention provides, also, an improved process for scrubbing hot chlorination gases obtained by the chlorination of oxidic titaniferous materials which does not have the disadvantages of the two types of processes discussed heretofore. A further object of the invention is to provide a process for the treatment of hot gases produced by the chlorination of oxidic titaniferous raw materials which continuously yields titanium tetrachloride in gaseous phase essentially free of suspended solids in an amount at least equaling that produced by the chlorination by continuously contacting the chlorination gases with an amount of liquid titanium tetrachloride sufficient to condense and wash out substantially all of the normally solid matter in liquid residual titanium tetrachloride which can be removed as a free flowing liquid body thereby avoiding clogging of the apparatus and the resulting interruption of the continuity of the process.

In accordance with the process of this invention, the gases produced in the chlorinator are passed through a cooling tower or heat exchanger where they are intimately contacted with liquid titanium tetrachloride having a desired temperature and in an amount, in excess of that vaporized by the hot chlorination gases, which condenses normally solid metallic chlorides but is insufficient to result in a net condensation of titanium tetrachloride from the chlorination gases. In other words, the amount of gaseous titanium tetrachloride coming out of the heat exchanger always at least equals the amount produced in the chlorinator. The amount of liquid titanium tetrachloride, used in excess of that vaporized, is regulated such that sufficient residual liquid is provided to wash out the condensed normally solid chlorides and contaminating solid matter suspended in the hot chlorination gases, if any, as a free flowing liquid body which is readily removed from the condenser without danger of clogging the apparatus. The amount of residual titanium tetrachloride should substantially exceed the amount of solid matter collected in the condenser. The required amount of liquid titanium tetrachloride can be determined by a skilled operator as it depends on the temperature and the composition of the chlorination gases at the inlet of the heat exchanger and on the temperatures of the liquid titanium tetrachloride which one plans to use for washing, sprinkling or otherwise intimately contacting the chlorination gases.

The temperature of the liquid titanium tetrachloride used for washing chlorination gases may vary within rather wide limits. Normally the temperature used will fall between 0° and 136° C., which is the ebullition point of the titanium tetrachloride, but preferably is between about 70° and 130° C. An amount of liquid titanium tetrachloride, at a desired temperature within the stated temperature range, can readily be selected so that the amount of gaseous  $TiCl_4$  coming out of the condenser is at least equal the amount introduced by the chlorination gases while sufficient residual excess liquid  $TiCl_4$  remains to substantially exceed the amount of condensed solid chlorides. In this way, normally solid matter is removed from the chlorination gases without danger of clogging and purified chlorination gases come out of the condenser saturated with titanium tetrachloride vapors.

When one operates without the limits of this invention one falls within the types of previously suggested processes discussed herein with all their disadvantages.

In the actual practice of this invention it has been demonstrated that it is always possible to select an amount of liquid titanium tetrachloride, within the scope of this invention, which will enable one to select a simple tower serving both as a heat exchanger and gas scrubber without any clogging taking place in the apparatus. In particular, experience has shown that the liquid titanium tetrachloride containing up to 30% of solid materials, such as  $FeCl_3$ ,  $FeCl_2$ ,  $AlCl_3$ , oxidic chlorides, dust, etc. is a free flowing liquid body which can be easily removed from the apparatus. More particularly, according to this invention, chlorination gases are caused to flow through a heat exchange zone where they are scrubbed or washed with liquid titanium tetrachloride, at any desired temperature, in an amount such that the liquid effluent obtained after cooling the chlorination gases contains less than 30-40% of solids and such that  $TiCl_4$  comes out as gaseous vapors in an amount at least equal to that introduced by the chlorination gases. In this way the chlorination gases are washed by an amount of liquid titanium tetrachloride which is sufficient to remove all of the condensed solid chlorides without the risk of clogging the apparatus.

The attached graphs, designated as Fig. 1 and Fig. 2, showing curves representing chlorination gases washed with an amount of liquid titanium tetrachloride within and without the scope of the invention, will facilitate an understanding of the invention. In these graphs the temperatures of the liquid titanium tetrachloride used for washing the chlorination gases are plotted as the abscissa and the amount of liquid titanium tetrachloride in kgs. per unit of time per 100 kg. of gaseous titanium tetrachloride introduced by the chlorination gases are plotted on a logarithmic scale as the ordinates.

The curves of Fig. 1 refer to chlorination gases obtained from rutile having the following analysis:

|               | Percent |
|---------------|---------|
| $TiO_2$       | 96      |
| $FeO-Fe_2O_3$ | 3       |
| $SiO_2$       | 1       |

The gases are assumed to enter the condenser at a temperature of 800° C. and to have a titanium tetrachloride initial condensation point, or dew-point, of 100° C.

Curve I represents the maximum flow of sprinkling or washing titanium tetrachloride in the heat exchanger, expressed as a function of the temperature of the liquid titanium tetrachloride, such that it is completely volatilized by heat exchange with the gases from the chlorinator.

Curve II represents a flow of an amount of liquid titanium tetrachloride through the heat exchanger, also expressed as a function of the temperature of the liquid titanium tetrachloride, such that the amount of titanium tetrachloride contained in the gases flowing from the condenser just equals the amount of titanium tetrachloride contained in the chlorination gases entering the

condenser. In other words, curve II represents the conditions under which there is no net vaporization of the liquid titanium tetrachloride introduced into the condenser.

- 5 Curve III represents a flow of an amount of liquid titanium tetrachloride into the heat exchanger for heat exchange with the chlorination gases such that the effluent liquid titanium tetrachloride contains not more than 30% of solids.
- 10 Curves IV, V and VI, of Fig. 2, are curves corresponding respectively to curves I, II and III of Fig. 1, but represent chlorination gases, coming into the exchanger at 800° C. obtained from ilmenite ore of the following composition:

|                                                      | Percent |
|------------------------------------------------------|---------|
| $TiO_2$                                              | 52      |
| $FeO-Fe_2O_3$                                        | 46      |
| ( $\frac{1}{3}$ ferric Fe, $\frac{2}{3}$ ferrous Fe) |         |
| $SiO_2$                                              | 1       |

The  $TiCl_4$  dew-point of these gases is 90° C.

Other ores, ore mixtures, or concentrates when used in the chlorinator, other temperatures at which the gases are introduced into the heat exchanger and other  $TiCl_4$  dew-points of such gases will give curves similar to those of the two specific illustrative examples.

- 25 In each case the three curves discussed above will delimit three principal zones A, B and C. As shown in the two attached drawings, zone A below curve I or curve 30 IV, corresponds to the known methods using restricted sprinkling or spraying with small amounts of  $TiCl_4$  as described earlier herein as a type "b," zone C above curve II or curve V corresponds to the methods relying upon extensive condensation of vapors so that less  $TiCl_4$  35 in the vapor state comes out of the heat exchanger than is introduced with the chlorinated gases as discussed also earlier herein as type "a."

Zone B included between curves I and II or IV and V is the zone within which this invention operates, namely, 40 a zone between curve II and a curve approximating curve I or a zone between curve V and a curve approximating curve IV where the amount of residual liquid  $TiCl_4$  is sufficient to carry any solids collected therein. It is preferred to remain substantially above curve I or 45 curve IV, i. e. between curves III and II or between curves VI and V so that the proportion of solid chloride in the residual liquid  $TiCl_4$  is less than 30 to 40%.

The advantages of such a method are as follows:

- 50 A. An amount of  $TiCl_4$  comes out of the heat exchanger as a vapor completely washed and cleaned in an amount which is at least equal to the amount of  $TiCl_4$  produced in the chlorinator.
- B. The solid chlorides are condensed and eliminated at the bottom of the heat exchanger in a very simple manner which can easily be made continuous.

C. The condenser for recovering the  $TiCl_4$  vapors acts upon clean vapor so that one is able to use a condenser of an ordinary type, which is dependable and costs little.

D. The condenser for recovering the  $TiCl_4$  vapors acts 60 upon saturated vapors and therefore with a high coefficient of heat exchange. In this way a small apparatus may be used and the investment costs are accordingly reduced.

E. The quantity of contacting liquid  $TiCl_4$  within the 65 scope of this invention can be relatively small, advantageously in the neighborhood of the lower limit which insures good removal of the condensed solid chlorides. In this way the heat exchanger can also be of a small size and, therefore relatively inexpensive.

F. The heat exchanger can be a simple exchanger of 70 conventional type, for example, either tubular, or a heat exchanger filled with packing rings. This is a very important feature of the invention. Actually the continuous scrubbing of the gases eliminates all risk of clogging and, 75 the utilization of the heat of vaporization of the added

liquid  $TiCl_4$ , permits a highly efficient operation and consequently a small size apparatus can be used.

G. The liquid impure or contaminated residual  $TiCl_4$  flows out of the heat exchanger almost at its boiling point and the amount thereof can be reduced to the minimum necessary for flowing out the condensed solid chlorides. Both of these features result in a saving of heat.

According to an important embodiment of the invention, it is preferable to work with hot  $TiCl_4$  for contacting or scrubbing the chlorination gases, i. e. liquid  $TiCl_4$  at or above about 70-80° C. Good results, however, are obtained by using liquid  $TiCl_4$  having a temperature of, say 30-80° C. Actually for a given amount of  $TiCl_4$  used for contacting the chlorination gases, the warmer the  $TiCl_4$  the more readily it vaporizes and consequently the smaller size of the apparatus required. At preferred temperatures when one works with liquid  $TiCl_4$  having a temperature in the neighborhood of 100 to 136° C. the heat exchange is practically reduced to the latent heat of vaporization and the process becomes automatic with respect to temperature controls.

Furthermore, the invention provides for all or part of the alternatives given below which can be used separately or in combination:

(a) The heat exchanger may be a column or tower in which the gases flow countercurrent to the washing  $TiCl_4$  and the column may be filled or packed with simple filling or surface extending materials, for instance, Rasching rings, thereby assuring extended contact between the gases and the liquid  $TiCl_4$  and the necessary amount of heat exchange surface.

(b) Part, at least, of the  $TiCl_4$  coming out of the heat exchanger as vapor may be condensed and returned to the exchanger to serve for spraying or otherwise intimately contacting the hot gases with liquid  $TiCl_4$ .

(c) Residual impure  $TiCl_4$  may be separated and at least part thereof, after separating impurities, returned to the exchanger to serve for scrubbing the hot gases.

(d) The separation of the purified residual liquid  $TiCl_4$  may be preferably accomplished by distillation and condensation with the removal of occluded gases.

(e) By addition of any of known appropriate purifying agents, such as oil, for instance, to the residual  $TiCl_4$  a further purification of the  $TiCl_4$  may be simultaneously obtained.

(f) The  $TiCl_4$  product may be and preferably is taken in part, at least, from the residual liquid  $TiCl_4$  after separation from its impurities.

The invention has as a particularly desirable embodiment, a cyclic process for the preparation of  $TiCl_4$  involving passing the gases coming from a chlorinator through a heat exchanger where they are scrubbed or sprayed with liquid  $TiCl_4$ , preferably hot liquid  $TiCl_4$ , at a rate between the limits hereinbefore defined, condensing the  $TiCl_4$  coming out as vapor, separating the residual liquid  $TiCl_4$  flowing through the heat exchanger and returning to the heat exchanger the  $TiCl_4$  thus obtained diminished by the net production of  $TiCl_4$ . The net production of  $TiCl_4$  can either be taken from the condensed  $TiCl_4$  which comes out of the heat exchanger as vapor or preferably from the  $TiCl_4$  separated from the residual liquid  $TiCl_4$  or from both.

On the attached drawings, two examples of apparatus suitable for use in the practice of the invention are shown diagrammatically.

Fig. 3 is a diagrammatic representation of one embodiment of the invention in which the heat exchanger is shown in vertical section.

Fig. 4 is a diagrammatic representation of an arrangement suitable for the practice of a cyclic process according to the invention, constituting a second embodiment, various elements being shown in vertical section.

In Fig. 3, exchanger 1 is provided with packing rings 10. Gases containing a quantity Q of  $TiCl_4$  from a chlorinator are introduced into heat exchanger 1 through

conduit 2, and liquid  $TiCl_4$ , at the rates previously discussed, are introduced into the top of the heat exchanger 1 through conduit 3. Residual gases containing vapors of  $TiCl_4$  in a quantity at least equaling Q flow out of the heat exchanger 1 through conduit 4 into condenser 5. The residual  $TiCl_4$  carrying impurities flows out conduit 6. The quantity of  $TiCl_4$  used for contacting the chlorination gases preferably is such that the solid impurities are less than 30% of the residual  $TiCl_4$ .

Fig. 4 illustrates an arrangement for practicing a cyclic process in accordance with the invention. The following example using this arrangement will further illustrate the invention:

*Example*

15 Rutile chlorination gases coming from chlorinator 7 flow through conduit 2 into heat exchanger 1, which is insulated and provided with Rasching rings 10.

The chlorination gases possess the following characteristics:

|    |                                                                     |                         |
|----|---------------------------------------------------------------------|-------------------------|
| 20 | Temperature                                                         | 800° C.                 |
|    | Dew-point                                                           | 110° C.                 |
|    | Quantity of $TiCl_4$ in the gases                                   | 500 kgs./h.             |
|    | Chlorination gases at 800° C.                                       | 776 m. <sup>3</sup> /h. |
| 25 | Corresponding amount of solids                                      | 25 kgs./h.              |
|    | Sensible heat of the chlorination gases between 800° C. and 110° C. | 66,000 kc./h.           |

The characteristics of the heat exchange tower 1 are:

|    |                           |          |
|----|---------------------------|----------|
| 30 | Diameter of the tower     | mm 430   |
|    | Height                    | mm 3500  |
|    | Size of the filling rings | mm 30/30 |

The liquid  $TiCl_4$  introduced in 3a, 3b, has the following characteristics:

|    |                                        |                                                               |
|----|----------------------------------------|---------------------------------------------------------------|
| 35 | Temperature of the liquid for spraying | 100° C.                                                       |
|    | Spraying rate                          | 2,420 kgs./h. (1500 kgs. through 3a and 920 kgs. through 3b). |

In condenser 5, one condenses clean  $TiCl_4$ , of which about 1500 kgs./h. flows back into the exchanger through 3a.

Through conduit 6, 920 kgs./h. of  $TiCl_4$  are flowed, carrying solid impurities at a concentration of 2.62% (less than 30%). The net production is then collected at B.

The working characteristics are:

|    |                                    |                                          |
|----|------------------------------------|------------------------------------------|
| 50 | Apparent linear speed of the gases | 1.5 m./sec.                              |
|    | Head spraying                      | 10.5 m. <sup>3</sup> /m. <sup>2</sup> /h |
|    | Bottom outflow                     | 4 m. <sup>3</sup> /m. <sup>2</sup> /h.   |
|    | Pressure loss in the exchanger     | less than 50 mm. water.                  |

All these quantities are conventionally employed in industrial processes.

The  $TiCl_4$  coming out as vapor through conduit 4 is condensed in condenser 5 and the residual gases are removed through conduit 8 at about 20° C., for example. Condensed  $TiCl_4$ , in the neighborhood of 110° C., flowing through conduit 9 is returned to the exchanger, except such part of the condensed  $TiCl_4$  as is taken off at B.

The impure residual  $TiCl_4$  flowing out through conduit 6, at about 110° C., flows into evaporator 11 containing a heating element 12. The evaporator is supplied with oil for purifying the liquid  $TiCl_4$  through conduit 13 and slurry is discharged through outlet 14 and sent to drum dryers or the like (not shown) in order to recover the  $TiCl_4$  entrained in the slurry. The  $TiCl_4$  flowing out through conduit 15 is condensed in the condenser 16 and residual gases are removed through conduit 17 at about 20° C., for example. After cooling at least a part of the  $TiCl_4$  liquefied in condenser 16 from about 136° C. to about 110° C. in cooler 18, it is passed through conduit 3b to the heat exchanger 1.

One can collect all or part of the net production at B.

Preferably, at least a part of the net production of  $TiCl_4$  is collected from the clean vapors recovered from the evaporator 11. For instance, purified liquid  $TiCl_4$  can be discharged at A from conduits 20 and 19 as an overflow from condenser 16. For example, 2000 kgs./h. of cleansed  $TiCl_4$  could be introduced through 3a and 420 kgs./h. through 3b.

If the ore treated is ilmenite and the same amount of liquid  $TiCl_4$  is used for washing the chlorination gases, the residual liquid  $TiCl_4$  would contain 35% of solid matter. Under such circumstances, one should reduce the solid content of the residual liquid  $TiCl_4$  to about 15% by washing with 3340 kgs./h.

The general advantages of the present invention have already been mentioned. The cyclic process, included purely for illustrative purposes, has these and certain other advantages, among which are the following:

1. Due to the fact that the exchanger 1 is supplied with liquid  $TiCl_4$  from apparatus elements which operate at constant temperatures (condenser 5 and cooler 18), the process is essentially continuous and practically fool-proof. As a result, only the quantity of  $TiCl_4$  in circulation need be varied to suit the nature of the chlorination gases, and this can be very easily regulated.

2. All of the equipment is completely air-tight thereby eliminating risks of contamination by moisture.

3. Mechanical devices for circulating fluids (pumps, etc.) are completely eliminated and consequently abrasion problems resulting in costly maintenance are likewise eliminated.

4. Through this process one can recover  $TiCl_4$  from chlorinated raw materials which are high in impurity content (especially iron).

5. The process can be absolutely continuous for the elimination of impurities.

6. The process provides for the possibility of adding oil or other products into the evaporator for purification of the residual  $TiCl_4$ .

7. The spraying and scrubbing liquid being clean, no clogging difficulties are encountered in the pipes and condensers.

8. In the spraying circuit used for collecting  $TiCl_4$  for washing the chlorination gases one can withdraw the  $TiCl_4$  when it is in the vapor state and rectify it to eliminate  $SiCl_4$ .

9. The invention enables one to achieve, through very simple and new means, the condensation of  $TiCl_4$  as it comes from the chlorinator and without the risk of the deposit of solid impurities; the process being in ultimate analysis a scrubbing of the  $TiCl_4$  vapors before their condensation.

It will be understood that gases obtained by the chlorination of oxidic titaniferous materials usually contain substances which are normally solid, normally liquid and normally gaseous at room temperatures and that such substances are referred to herein respectively as normally solid, normally liquid and normally gaseous substances.

While the foregoing specification sets forth numerous details and examples to illustrate the practice of this invention, it will be understood that they may be varied widely without departing from the spirit or the scope of the disclosed invention which is intended to be defined by the appended claims.

We claim:

1. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said

zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continuously taking off from said zone gases containing  $TiCl_4$  vapors in an amount at least equal to the amount thereof contained in said inflowing stream of hot gases, and removing from said zone in the outflowing metal chlorides substantially all the heat abstracted from said stream in said zone.

2. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$  at a temperature of 80° to 136° C., providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continuously taking off from said zone gases containing  $TiCl_4$  vapors in an amount at least equal to the amount thereof contained in said inflowing stream of hot gases, and removing from said zone in the outflowing metal chlorides substantially all the heat abstracted from said stream in said zone.

3. A process for continuously separating normally solid metal chloride from hot gases produced by the chlorination of oxidic titaniferous material, said gases containing substantially all the metallic chloride vapors produced in the chlorination, which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continuously taking off from said zone gases containing  $TiCl_4$  vapors in an amount at least equal to the amount thereof contained in said inflowing stream of hot gases, and removing from said zone in the outflowing metal chlorides substantially all the heat abstracted from said stream in said zone.

4. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continuously taking off from said zone gases containing  $TiCl_4$  vapors in an amount at least equal to the amount thereof contained in said inflowing stream of hot gases, removing from said zone in the outflowing metal chlorides substantially all the heat abstracted from said stream in said zone, con-

tinuously condensing  $TiCl_4$  from said offtake gases to obtain a liquid  $TiCl_4$  product, and returning at least a part of said product into said zone to continue said inflow of liquid  $TiCl_4$ .

5. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continually removing from said zone liquid  $TiCl_4$  containing solids collected in said zone, continuously taking off from said zone gases containing  $TiCl_4$  vapors in an amount at least equal to the amount thereof contained in said inflowing stream of hot gases, removing from said zone in the outflowing metal chlorides substantially all the heat abstracted from said stream in said zone, vaporizing  $TiCl_4$  from said liquid  $TiCl_4$  removed from said zone, condensing resulting vapors to obtain a liquid  $TiCl_4$  product, and returning at least a part of said liquid  $TiCl_4$  product into said zone to continue said liquid inflow.

6. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow such that a substantial amount of the liquid inflow is vaporized by the heat of said gases, continuously collecting the resulting condensed solids in said flow of liquid  $TiCl_4$  and washing them out of said zone therein, continuously taking off from said zone gases containing  $TiCl_4$  vapors in an amount substantially greater than the amount thereof contained in said inflowing stream of hot gases, and removing from said zone in the outflowing metal chlorides substantially all the heat abstracted from said stream in said zone.

7. A process for continuously separating normally solid metal chloride from hot gases containing mixed vapors of such chloride and  $TiCl_4$ , which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continually removing from said zone liquid  $TiCl_4$  containing solids collected in said zone, continuously taking off from said zone gases containing  $TiCl_4$  vapors in an amount at least equal to the amount thereof contained in said inflowing stream of hot gases, removing from said zone in the outflowing metal chlorides substantially all the heat abstracted from said stream in said zone, vaporizing  $TiCl_4$  from said liquid  $TiCl_4$  removed from said zone, condensing resulting vapors to obtain a liquid  $TiCl_4$  product, con-

tinuously condensing  $TiCl_4$  from said offtake gases to obtain another liquid  $TiCl_4$  product, and returning into said zone a quantity of said products sufficient to maintain said liquid inflow.

5. A process for continuously separating normally solid metal chloride from hot gases produced by the chlorination of oxidic titaniferous material, said gases containing substantially all of the metallic chlorides vaporized in the chlorination, which comprises continuously flowing a stream of said gases into a heat exchange zone, continuously contacting and scrubbing said gases in said zone with an inflow of liquid  $TiCl_4$ , providing in said liquid inflow an amount of  $TiCl_4$  at least sufficient by itself both to cool said stream below the condensation temperature of said normally solid chloride and to maintain a free flow of liquid  $TiCl_4$  through said zone, yet keeping the amount and temperature of said liquid inflow insufficient to cool said stream below the dew point of its  $TiCl_4$  content, continuously collecting the resulting condensed solids in said flow of liquid  $TiCl_4$  and washing them out of said zone therein, continually removing from said zone liquid  $TiCl_4$  containing solids collected in said zone, continuously taking off from said zone gases containing  $TiCl_4$  vapors in an amount at least equal to the amount thereof contained in said inflowing stream of hot gases, removing from said zone in the outflowing metal chlorides substantially all the heat abstracted from said stream in said zone, vaporizing  $TiCl_4$  from said liquid  $TiCl_4$  removed from said zone, condensing resulting vapors to obtain a liquid  $TiCl_4$  product, continuously condensing  $TiCl_4$  from said offtake gases to obtain another liquid  $TiCl_4$  product, returning into said zone substantially all said last mentioned product and sufficient of said first mentioned product to maintain said liquid inflow, and recovering the remainder of said first mentioned product as a liquid  $TiCl_4$  purified by the process.

9. A cyclic process for cooling and separating out normally solid components from hot gases produced by the chlorination of oxidic titaniferous material, said gases containing substantially all of the metallic chlorides vaporized in the chlorination, which comprises continuously flowing said gases through a heat exchange zone, continuously and intimately contacting them in said zone with a flow of liquid titanium tetrachloride to cool the gases and condense solids therein, the amount of said liquid titanium tetrachloride being such that there is a substantially greater amount of titanium tetrachloride vapors flowing out of said zone than introduced by said gases but such that a residual amount of liquid titanium tetrachloride flows out of said zone which contains not more than 30-40% solids collected therein, continuously removing a stream of residual titanium tetrachloride containing said solids, vaporizing at least a portion of the removed liquid titanium tetrachloride and next cooling and condensing the vapors to liquid titanium tetrachloride thereby obtaining purified residual liquid titanium tetrachloride, returning at least a part of the purified residual liquid titanium tetrachloride to the heat exchange zone to cool additional gases, continuously cooling the residual gases flowing out of said zone to form condensed liquid titanium tetrachloride, and returning into said zone a quantity of said condensed liquid titanium tetrachloride and purified residual liquid titanium tetrachloride sufficient to maintain said flow.

10. A cyclic process for cooling and separating out normally solid components from hot gases produced by the chlorination of oxidic titaniferous material, said gases containing in vapor phase substantially all of the metallic chloride, vaporized in the chlorination, which comprises continuously flowing said gases through a heat exchange zone, continuously and intimately contacting them in said zone with a flow of liquid titanium tetrachloride to separate solids from the gases, the amount of said liquid titanium tetrachloride being such that there is a

substantially greater amount of titanium tetrachloride vapors flowing out of said zone than introduced by said gases but such that a residual amount of free flowing liquid titanium tetrachloride flows out of said zone containing not more than 30-40% collected solids, continuously removing a stream of residual titanium tetrachloride containing said solids, continuously separating a purified residual liquid titanium tetrachloride from solids in said outflow of residual titanium tetrachloride apart from said heat exchange zone, continuously cooling the residual gases flowing out of said zone to form condensed liquid titanium tetrachloride, and returning into said zone most of the quantity of the condensed liquid titanium tetrachloride and purified residual liquid titanium tetrachloride to contact a further flow of gases.

11. A cyclic process for recovering titanium tetrachloride from hot gases produced by the chlorination of oxidic titaniferous material, said gases containing substantially all of the metallic chlorides vaporized in the chlorination, which comprises continuously flowing said gases through a heat exchange zone, continuously and intimately contacting them in said zone with a flow of liquid titanium tetrachloride to separate solids from the gases, the amount of said liquid titanium tetrachloride being such that there is a substantially greater amount of titanium tetrachloride vapors flowing out of said zone than introduced by said gases but such that a residual amount of liquid titanium tetrachloride flows out of said zone which contains not more than 30-40% solids collected therein, continuously removing a stream of residual titanium tetrachloride containing said solids, continuously vaporizing titanium tetrachloride from the removed residual titanium tetrachloride and next continuously condensing the vaporized residual titanium tetrachloride to form purified liquid residual titanium tetrachloride, continuously cooling the residual gases flowing out of said zone to form condensed liquid titanium tetrachloride, returning into said zone sufficient of the condensed liquid titanium tetrachloride and purified residual liquid titanium tetrachloride to maintain said flow, and recovering excess titanium tetrachloride not returned to said zone.

12. A continuous cyclic process for recovering titanium tetrachloride from hot gases produced by the chlorination of oxidic titaniferous material, said gases

containing substantially all of the metallic chlorides vaporized in the chlorination, which comprises continuously flowing said gases in a vertically disposed direction through a heat exchange zone provided with surface extending material, continuously and intimately contacting them in said zone with a counter current flow of liquid titanium tetrachloride to condense solids therein, the amount and temperature of said liquid titanium tetrachloride being such that there is a substantially greater amount of titanium tetrachloride vapors flowing out of said zone than introduced by said gases but such that a residual amount of liquid titanium tetrachloride flows out of said zone which contains not more than 30-40% solids collected therein, continuously removing a stream of residual titanium tetrachloride containing said solids, continuously vaporizing titanium tetrachloride from the removed residual titanium tetrachloride and next continuously condensing the vaporized residual titanium tetrachloride to form purified residual liquid titanium tetrachloride, continuously cooling the residual gases flowing out of said zone to form condensed liquid titanium tetrachloride, returning into said zone at the temperatures of said flow sufficient of the condensed liquid titanium tetrachloride and purified residual liquid titanium tetrachloride to maintain said flow, and recovering liquid titanium tetrachloride substantially free of dissolved solids from an excess of titanium tetrachloride not returned to said zone.

13. The process as described in claim 12, the counter current flow of liquid titanium tetrachloride being introduced into the heat exchange zone at a temperature of 100-136° C.

14. The process as described in claim 12, the flow of liquid titanium tetrachloride being introduced into the heat exchange zone not exceeding 10 times the weight of titanium tetrachloride vapors in the flow of said gases and the residual titanium tetrachloride flowing out of said zone containing more than 1% of solids.

#### References Cited in the file of this patent

#### UNITED STATES PATENTS

- |           |                   |                |
|-----------|-------------------|----------------|
| 2,675,890 | Frey et al. ----- | Apr. 20, 1954  |
| 2,718,279 | Kraus -----       | Sept. 20, 1955 |